



US005780154A

# United States Patent [19]

Okano et al.

[11] Patent Number: 5,780,154  
[45] Date of Patent: Jul. 14, 1998

[54] BORON NITRIDE FIBER AND PROCESS FOR PRODUCTION THEREOF

4-272231 9/1992 Japan.  
5-310404 11/1993 Japan.

[75] Inventors: **Yoshio Okano; Hiroya Yamashita**,  
both of Tsukuba, Japan

[73] Assignee: **Tokuyama Corporation**, Yamaguchi,  
Japan

[21] Appl. No.: 556,985

[22] PCT Filed: Mar. 20, 1995

[86] PCT No.: PCT/JP95/00500

§ 371 Date: Nov. 22, 1995

§ 102(e) Date: Nov. 22, 1995

[87] PCT Pub. No.: WO95/25834

PCT Pub. Date: Sep. 28, 1995

## [30] Foreign Application Priority Data

Mar. 22, 1994 [JP] Japan ..... 6-050779

[51] Int. Cl.<sup>6</sup> ..... B32B 9/00

[52] U.S. Cl. ..... 428/366; 428/364; 264/345;  
264/346; 501/95.1

[58] Field of Search ..... 428/364, 367,  
428/366; 509/95.1, 94.4; 264/345, 346

## [56] References Cited

### U.S. PATENT DOCUMENTS

3,668,059 6/1972 Economy et al. ..... 161/170  
4,707,556 11/1987 Paciorek et al. ..... 556/403  
5,061,469 10/1991 Kimura ..... 423/290

### FOREIGN PATENT DOCUMENTS

53-37837 10/1978 Japan.  
63-195173 8/1988 Japan.  
1-97213 4/1989 Japan.  
1-290510 11/1989 Japan.  
2-74614 3/1990 Japan.

## OTHER PUBLICATIONS

Fazen et al. "Thermally Induced Borazine Dehydropolymerization Reactions, Synthesis And Ceramic Conversion Reactions Of A New High-Yield Polymeric Precursor To Boron Nitride", *Chemistry of Materials*, vol. 2, 96-97 (1990).

Lynch et al., "Transition-Metal-Promoted Reactions Of Boron Hydrides. 10.<sup>1</sup> Rhodium-Catalyzed Syntheses Of B-Alkenylborazines", *Journal of American Chemical Society*, vol. 109, 5867-5868 (1987).

Rees, Jr., et al. "High-Yield Synthesis Of B<sub>4</sub>C/BN Ceramic Materials By Pyrolysis Of Polymeric Lewis Base Adducts Of Decaborane(14)", *Journal of America Ceramic Society*, vol. 71, C194 (1988).

Primary Examiner—Marion E. McCamish

Assistant Examiner—J. M. Gray

Attorney, Agent, or Firm—Wenderoth, Lind & Ponack

## [57] ABSTRACT

A boron nitride fiber comprising hexagonal and/or turbostratic boron nitride having C planes oriented substantially parallel to the fiber axis and a degree of orientation of 0.74 or above can be obtained by heating an adduct between a boron trihalide such as boron trichloride or the like and a nitrile compound such as acetonitrile, benzonitrile or the like, and an ammonium halide or a primary amine hydrohalide in the presence of a boron trihalide at around 125° C. to form a boron nitride precursor, dissolving the boron nitride precursor in a solvent such as N,N'-dimethyl formamide or the like, capable of dissolving the precursor, spinning the solution to obtain a boron nitride precursor fiber, heat-treating the precursor fiber in an inert gas atmosphere and then in an ammonia gas atmosphere to obtain a boron nitride fiber, and heat-treating the boron nitride fiber with a tensile stress being applied to the fiber. The boron nitride fiber of the present invention has a degree of orientation of 0.74 or above and therefore has a high tensile strength.

40 Claims, 2 Drawing Sheets



FIG. 1



FIG. 2





FIG. 3

## BORON NITRIDE FIBER AND PROCESS FOR PRODUCTION THEREOF

### TECHNICAL FIELD

The present invention relates to a boron nitride fiber and a process for production thereof.

More particularly, the present invention relates to a boron nitride fiber having a tensile strength larger than that of any boron nitride fiber known heretofore, as well as to a process for production of the fiber.

### BACKGROUND ART

Boron nitride fibers are known. None of known boron nitride fibers, however, has a sufficiently large tensile strength, and no boron nitride fiber having a sufficiently large tensile strength is known yet.

A boron nitride fiber having a sufficiently large strength can be used, for example, as a reinforcing fiber for ceramic material.

Ceramic materials, having a high strength and moreover being stable up to high temperatures, are expected to be applied as a high-temperature structural material which no plastic or metal material can replace. While the ceramic materials have excellent thermal and mechanical properties, they have inherent brittleness which causes cracking easily. Owing to this inherent brittleness of ceramic, fracture of ceramic takes place catastrophically. Therefore, the ceramic materials are not reliable for use as a structural material which must retain a given structure, and are not in wide use.

In order to overcome the brittleness of ceramic, it is effective to blend a ceramic with a reinforcing material to convert the ceramic into a composite material having an improved toughness. As the reinforcing material, there have been studied spherical particles, platy particles, whiskers, continuous fibers, etc. It is particularly effective to blend a ceramic with a continuous fiber for improved toughness, and it is known that the method can increase the fracture toughness of a ceramic to about the same level as that of aluminum alloy. Prospective continuous fibers used as a reinforcing material for converting a ceramic into a composite material are ceramic fibers (e.g. a silicon carbide fiber and an alumina fiber) and a carbon fiber.

Both the ceramic fibers and the carbon fiber, however, have respective drawbacks and are not fully satisfactory as a fiber used as a reinforcing material for converting a ceramic into a composite material. For example, the ceramic fibers, which have a polycrystalline structure consisting of fine crystals, come to possess a significantly reduced tensile strength caused by the growth of the crystals when the ceramic fibers are exposed to high temperatures. In general, when a reinforcing fiber is blended with a ceramic to obtain a composite material, it is necessary to heat them at a high temperature of one thousand and several hundred degrees (centigrade) or above. As a result, a ceramic fiber, when used as a reinforcing material for ceramic to obtain a composite material, causes reduction in tensile strength during the process for obtaining the composite material and it is difficult to obtain a composite material of improved toughness.

Meanwhile, the carbon fiber exhibits little structural change at high temperatures and retains its tensile strength even when heated to about 2,000° C. Consequently, after the heat treatment to obtain a carbon fiber reinforced ceramic matrix composite, the carbon fiber can retain its strength, which makes it possible to use a carbon fiber as a reinforcing

material for ceramic matrix composite material of improved toughness. However, the carbon fiber is oxidized and loses its weight in air at temperatures of about 400° C. or above; therefore, the resulting carbon fiber-reinforced ceramic cannot be used at high temperatures in air or in an oxidizing atmosphere.

Thus, there is not yet developed any reinforcing fiber capable of reinforcing a brittle material (e.g. ceramic) and endowing the material with high toughness without impairing the useful properties of the material.

In contrast, a boron nitride fiber, when containing no impurity (e.g. boron oxide) which promotes crystal growth, hardly exhibits structural change (e.g. grain growth of crystals) even at high temperatures and is presumed to give little reduction in tensile strength when exposed to high temperatures. That is, the reduction in tensile strength of boron nitride fiber caused by an exposure to high temperatures is presumed to be smaller than that of ceramic fiber. Moreover, the boron nitride is stable to oxidation in air up to about 1,000° C. and, as compared with a carbon fiber, has superior oxidation resistance.

In addition to the excellent heat resistance and oxidation resistance, the boron nitride fiber has excellent properties when used as a reinforcing fiber for obtaining a composite material. For example, the boron nitride has low reactivity with other substances, as appreciated from the fact that it is used as a material for crucibles or as a releasing agent. Therefore, it is thought that when combined with various ceramics, the boron nitride does not react with any matrix phase and can give a composite material.

The reason why a brittle material such as ceramic or the like can improve its fracture toughness when blended with a continuous fiber to convert into a composite material, is presumed to be that the mechanical energy applied to the composite material is absorbed by a "pull-out" phenomenon that the reinforcing fiber is pulled out from the matrix phase of the composite material at around the crack tip. The boron nitride fiber, having low reactivity with the matrix phase as mentioned above, does not bond to the matrix phase strongly in many cases. In addition, since the boron nitride fiber, has excellent solid lubricating properties, it is presumed that, when the boron nitride fiber is used as a reinforcing fiber to obtain a composite material, the "pull-out" phenomenon takes place easily and large improvement in fracture toughness can be obtained.

The promotion of "pull-out" by weak bonding to matrix phase and solid lubricating properties and consequent improvement in fracture toughness as mentioned above is expected also in a carbon fiber. However, the conditions under which the carbon fiber can be used, are restricted, for example, because it undergoes oxidation and dissipation in air at about 500° C. and because it has a high electrical conductivity.

Meanwhile, when a ceramic fiber such as alumina fiber, mullite fiber, silicon carbide fiber, silicon nitride fiber or the like is combined with a brittle material such as ceramic or the like to obtain a composite material, the bonding between the matrix phase and the fiber is strong in many cases. As a result, the "pull-out" phenomenon hardly occurs in such a composite material and no improvement in fracture toughness is obtained in many cases.

Also, the boron nitride fiber has, in addition to the above-mentioned properties when used as a reinforcing fiber, excellent properties such as high electrical resistance, high thermal shock resistance, high thermal conductivity and the like, leading to a material of high industrial utility.

For production of a boron nitride fiber, there is known a process which comprises spinning a boron nitride precursor containing boron and nitrogen and then heat-treatment of the resulting boron nitride precursor fiber to be pyrolyzed and converted into a boron nitride fiber (the process may hereinafter be referred to as precursor process); and a process which comprises heat-treatment of a boron oxide fiber in an ammonia atmosphere to nitride the fiber (this process may hereinafter be referred to as nitriding process).

As the precursor process among the processes for production of boron nitride fiber, there are known processes which comprise spinning a precursor fiber from a polycondensate of borazine or borazine derivative and then heat-treating the precursor fiber [Japanese Patent Publication No. 37837/1978, Japanese Patent Application Kokai (Laid-Open) No. 195173/1988, U.S. Pat. No. 5,061,469, U.S. Pat. No. 4,707,556, Chemistry of Materials, Vol. 2, 96-97 (1990), or Journal of American Chemical Society, Vol. 109, 5867-5868 (1987)]; and a process which comprises spinning a precursor fiber from a borane-amine adduct and then heat-treating the precursor fiber [Journal of American Ceramic Society, Vol. 71, C194 (1988)]. Of the boron nitride fibers obtained in these precursor processes, only those obtained in Japanese Patent Publication No. 37837/1978, Japanese Patent Application Kokai (Laid-Open) No. 195173/1988 and U.S. Pat. No. 5,061,469 (none of these fibers is subjected to any thermal stretching treatment under the application of a tensile stress) are measured for tensile strength, and their tensile strengths are 784 MPa, 500 MPa and 1,200 MPa, respectively. These tensile strengths are low as compared with, for example, the tensile strength 3,000 MPa or above of a carbon fiber. No particular means for increasing the tensile strengths is indicated in the above three literatures. In other precursor processes, only the possibility of boron nitride fiber production is described and no examination is made on the properties (e.g. tensile strength) of the boron nitride fiber obtained.

Meanwhile, in the process which comprises heat-treating a boron oxide fiber in an ammonia atmosphere to nitride the fiber to obtain a boron nitride fiber (U.S. Pat. No. 3,668,059), it is indicated that by partly nitriding a boron oxide fiber and subjecting the partly nitrided boron oxide fiber to thermal stretching and nitriding simultaneously, a boron nitride fiber of improved tensile modulus of elasticity can be obtained. The literature gives no detailed reason for this improved tensile modulus of elasticity but points out the small diameter of fiber resulting from thermal stretching, as an important factor of improved modulus. The tensile modulus of elasticity of this boron nitride fiber, however, is not significantly improved as compared with the tensile modulus of elasticity of the boron nitride fiber obtained by the precursor process. Also in this boron nitride fiber, the maximum tensile strength shown in Examples is 580 MPa although the fiber is stretched and has a diameter as small as 6  $\mu$ m or less, and is not significantly improved as compared with the tensile strength of the boron nitride fiber obtained by the precursor process. Thus, although many studies such as mentioned above have been made, the boron nitride fibers obtained heretofore have no sufficient tensile strength for reinforcement of brittle material; moreover, means for obtaining a boron nitride fiber of high strength are not yet developed and the research therefor has been stagnant.

#### DISCLOSURE OF THE INVENTION

Hence, an object of the present invention is to provide a boron nitride fiber having a large tensile strength.

A further object of the present invention is to provide a process for producing a boron nitride fiber having a large tensile strength.

According to the present invention, the former object can be achieved by a boron nitride fiber comprising boron nitride having a multi-layered structure consisting of planes (C planes) each formed by linkage of 6-membered rings in the plane, in which boron and nitrogen are positioned alternately and bonded to each other, which fiber has a tensile strength of at least 1,400 MPa.

According to the present invention, the former object can also be achieved by a boron nitride fiber comprising boron nitride having a multi-layered structure consisting of planes (C planes) each formed by linkage of 6-membered rings in the plane, in which boron and nitrogen are positioned alternately and bonded to each other, in which fiber at least part of each C plane is oriented substantially parallel to the fiber axis and the degree of orientation of each C plane is at least 0.74.

According to the present invention, the latter object can be achieved by a process for producing a boron nitride fiber, which comprises:

- 10 (a) reacting a boron trihalide-nitrile compound adduct with an ammonium halide or a primary amine hydrohalide in the presence of a boron trihalide to form a boron nitride precursor.
- 15 (b) dissolving the boron nitride precursor in a solvent to prepare a boron nitride precursor solution.
- 20 (c) spinning the boron nitride precursor solution to form a boron nitride precursor fiber.
- 25 (d) preheating the boron nitride precursor fiber in an inert gas atmosphere at 100°-600° C..
- 30 (e) treating the preheated fiber by ammonia in an ammonia gas atmosphere at 200°-1,300° C., and
- 35 (f) heating the fiber treated by ammonia in an inert gas atmosphere at 1,600°-2,300° C. with a tensile stress being applied to the fiber.

According to the present invention, the latter object can also be achieved by a process for producing a boron nitride fiber, which comprises:

- 40 (a) reacting a boron trihalide-nitrile compound adduct with an ammonium halide or a primary amine hydrohalide in the presence of a boron trihalide to form a boron nitride precursor.
- 45 (b) dissolving the boron nitride precursor and an acrylonitrile polymer in a solvent to prepare a boron nitride precursor solution.
- 50 (c) spinning the boron nitride precursor solution to form a boron nitride precursor fiber.
- 55 (d) preheating the boron nitride precursor fiber in an inert gas atmosphere at 100°-600° C..
- (e) treating the preheated fiber by ammonia in an ammonia gas atmosphere at 200°-1,300° C., and
- (f) heating the fiber treated by ammonia in an inert gas atmosphere at 1,600°-2,300° C. with a tensile stress being applied to the fiber.

#### BRIEF DESCRIPTION OF THE DRAWINGS

FIG. 1 is a photograph of a diffraction pattern obtained when a boron nitride fiber of the present invention obtained by heating an ammonia-treated boron nitride fiber in a nitrogen gas atmosphere at 1,800° C. with a tensile stress being applied to the fiber, was irradiated with an X-ray from a direction perpendicular to the fiber axis.

FIG. 2 is a photograph of a diffraction pattern obtained when a boron nitride fiber not falling in the present invention obtained by heating an ammonia-treated boron nitride fiber

in a nitrogen gas atmosphere at 1,800° C. with no tensile stress being applied to the fiber, was irradiated with an X-ray from a direction perpendicular to the fiber axis.

FIG. 3 shows an infrared absorption spectrum by KBr method, of a boron nitride fiber of the present invention.

#### BEST MODE FOR CARRYING OUT THE INVENTION

The present inventors made an extensive study from various angles in order to achieve the above objects. As a result, the inventors found a boron nitride fiber comprising hexagonal, rhombohedral and/or turbostratic boron nitride having C planes predominantly oriented to a direction parallel to the fiber axis, and further found for the first time that as the orientation of the boron nitride fiber becomes higher, the tensile strength of the fiber increases remarkably. The present invention has been completed based on the finding.

The present invention relates to a boron nitride fiber as well as to a process for production of the fiber.

That is, the present invention resides in a boron nitride fiber comprising boron nitride having a multi-layered structure consisting of planes (C planes) each formed by linkage of 6-membered rings in the plane, in which boron and nitrogen are positioned alternately and bonded to each other, which fiber has a tensile strength of at least 1,400 MPa.

The present invention resides also in a boron nitride fiber comprising boron nitride having a multi-layered structure consisting of planes (C planes) each formed by linkage of 6-membered rings in the plane, in which boron and nitrogen are positioned alternately and bonded to each other, in which fiber at least part of each C plane is oriented substantially parallel to the fiber axis and the degree of orientation of each C plane is at least 0.74.

Further, the present invention resides in a process for producing a boron nitride fiber, which comprises:

- (a) reacting a boron trihalide-nitrile compound adduct with an ammonium halide or a primary amine hydrohalide in the presence of a boron trihalide to form a boron nitride precursor,
- (b) dissolving the boron nitride precursor in a solvent to prepare a boron nitride precursor solution,
- (c) spinning the boron nitride precursor solution to form a boron nitride precursor fiber,
- (d) preheating the boron nitride precursor fiber in an inert gas atmosphere at 100°-600° C.,
- (e) treating the preheated fiber by ammonia in an ammonia gas atmosphere at 200°-1,300° C., and
- (f) heating the fiber treated by ammonia in an inert gas atmosphere at 1,600°-2,300° C. with a tensile stress being applied to the fiber.

Further, the present invention resides also in a process for producing a boron nitride fiber, which comprises:

- (a) reacting a boron trihalide-nitrile compound adduct with an ammonium halide or a primary amine hydrohalide in the presence of a boron trihalide to form a boron nitride precursor,
- (b) dissolving the boron nitride precursor and an acrylonitrile polymer in a solvent to prepare a boron nitride precursor solution,
- (c) spinning the boron nitride precursor solution to form a boron nitride precursor fiber,
- (d) preheating the boron nitride precursor fiber in an inert gas atmosphere at 100°-600° C.,

- (e) treating the preheated fiber by ammonia in an ammonia gas atmosphere at 200°-1,300° C., and
- (f) heating the fiber treated by ammonia in an inert gas atmosphere at 1,600°-2,300° C. with a tensile stress being applied to the fiber.

The above boron nitride fiber and process for production of the fiber, according to the present invention are herein-after described in detail.

Boron nitride is a substance formed by the chemical bonding of boron of the group III of periodic table and nitrogen of group V of the periodic table. The following two kinds of boron nitrides are known currently:

- (1) boron nitride having a structure in which boron and nitrogen are bonded to each other three-dimensionally, and
- (2) boron nitride having a structure in which boron and nitrogen are bonded to each other two-dimensionally.

As the boron nitride having a structure in which boron and nitrogen are bonded to each other two-dimensionally, there is known boron nitride having a multi-layered structure consisting of planes each formed by linkage of 6-membered rings in the plane in which boron and nitrogen are positioned alternately and bonded to each other.

As the boron nitride having a multi-layered structure consisting of the above-mentioned planes, the following three boron nitrides are known:

- (a) hexagonal boron nitride (h-BN) having a multi-layered structure consisting of two-layered structural units,
- (b) rhombohedral boron nitride (r-BN) having a multi-layered structure consisting of three-layered structural units, and
- (c) turbostratic boron nitride (t-BN) having a multi-layered structure wherein layers (planes) are not piled up regularly.

The boron nitride fiber of the present invention comprises the above-mentioned boron nitride having a multi-layered structure consisting of planes each formed by linkage of 6-membered rings in the plane in which boron and nitrogen are positioned alternately and bonded to each other.

The boron nitride according to the present invention, therefore, may comprise hexagonal boron nitride (h-BN), rhombohedral boron nitride (r-BN) and/or turbostratic boron nitride (t-BN).

Generally in the present invention, however, hexagonal boron nitride (h-BN) and/or turbostratic boron nitride (t-BN) constitutes the major part of the whole boron nitride in many cases and the proportion of rhombohedral boron nitride (r-BN), even if it is present, is small in many cases.

The hexagonal structure and rhombohedral structure have a structure in which the planes formed by two-dimensional linkage of 6-membered rings in which boron and nitrogen are positioned alternately and bonded to each other (the planes are herein-after referred to as "C planes" in some cases), are piled up regularly. The turbostratic structure is a structure in which the C planes are piled up without having any regularity in a direction perpendicular to the planes, and is called a structure consisting of randomly piled layers, in some cases.

Hexagonal boron nitride and turbostratic boron nitride can each be confirmed from the peak of diffraction from the (002) plane when subjected to X-ray diffractometry. The two crystal structures can be distinguished by examining, by X-ray diffractometry, a peak of diffraction from the crystal planes of boron nitride perpendicular to the C planes, for example, a peak of diffraction from the (110) plane. However, detection of such a diffraction peak [e.g. (110)

peak] to distinguish the hexagonal structure and the turbostratic structure is difficult, in some cases, when the crystallite size of boron nitride is very small as in the case of the boron nitride constituting the boron nitride fiber of the present invention, because the diffraction peak obtained by powder X-ray diffractometry has a very large width. Therefore, the boron nitride fiber of the present invention contains at least either of hexagonal boron nitride and turbostratic boron nitride, and is a mixture of hexagonal boron nitride and turbostratic boron nitride in some cases.

In the boron nitride fiber of the present invention, the crystallite size of the hexagonal boron nitride and turbostratic boron nitride constituting the fiber is very small, in the range of 10-60 Å.

The crystallite size represents the size of the hexagonal and/or turbostratic boron nitride constituting the boron nitride fiber, in a direction in which the C planes are piled up. Since in the hexagonal and/or turbostratic boron nitride the distance between two adjacent C planes is about 3.3 Å, crystallite size of 10-60 Å indicate that the boron nitride has a multi-layered structure consisting of 3-20 C planes and that such a boron nitride constitutes the boron nitride fiber of the present invention.

The boron nitride fiber of the present invention exhibits substantially no increase in crystallite size even when exposed to high temperatures. It is generally known that hexagonal boron nitride, when containing boron oxide as an impurity, exhibits an increase in crystallite size when heated at high temperatures. In the present invention, a boron nitride fiber having very small crystallite size is obtained, and the reason therefor is presumed to be that no oxygen is contained in the starting materials or introduced during the production process and consequently a boron nitride fiber can be produced which contains no boron oxide.

In the boron nitride fiber of the present invention, the most important matter is that the C planes of the hexagonal or turbostratic boron nitride constituting the fiber are predominantly oriented in a direction parallel to the fiber axis.

In the boron nitride fibers obtained heretofore, the C planes of the hexagonal or turbostratic boron nitride constituting each fiber are distributed isotropically to the fiber axis. Meanwhile, the present inventors found a boron nitride fiber in which the C planes of the hexagonal or turbostratic boron nitride constituting the fiber are oriented parallel to the fiber axis. The present inventors further found for the first time that an increase in degree of this orientation gives a boron nitride fiber having an increased tensile strength. The inventors are unable to make clear explanation of the reason why the orientation of the C planes of hexagonal or turbostratic boron nitride, parallel to fiber axis gives a boron nitride fiber having an increased tensile strength. However, the reason is presumed to be as follows.

In hexagonal or turbostratic boron nitride, the bond within each C plane is presumed to be mainly a covalent bond which is strong, and the bond between C planes is presumed to be mainly a bond by van der Waals force which is weak. Hence, it is presumed that an increase in the proportion of the strong bond within each C plane parallel the fiber axis gives an increased tensile strength. When the C planes of hexagonal or turbostratic boron nitride constituting a boron nitride fiber are oriented isotropically to the fiber axis, it is presumed that the tensile strength of the boron nitride fiber is suppressed by the presence of boron nitride whose C planes are perpendicular to the fiber axis, making it difficult to obtain a boron nitride fiber having a high tensile strength. This presumption is supported by the fact that a higher orientation of C planes of hexagonal or turbostratic boron nitride in a direction parallel to the fiber axis gives a higher strength.

In the past researches on boron nitride fibers, attention was paid only to the production of fibrous boron nitride and no attention was paid to the crystal orientation of boron nitride or to the effect of crystal orientation on properties (e.g. tensile strength) of boron nitride.

In expressing the distribution of the orientation of C planes of hexagonal or turbostratic boron nitride of boron nitride fiber to the fiber axis, degree of orientation of C planes (hereinafter referred to as "degree of orientation", in some cases) is used as the yardstick of the orientation distribution. The boron nitride fiber of the present invention has, as its feature, a degree of orientation of 0.74 or above. The present inventors also found a boron nitride fiber having a degree of orientation of less than 0.74 and it is possible to produce such a boron nitride fiber. Boron nitride fibers of various degrees of orientation were produced and the relation between the tensile strength and the degree of orientation, of these boron nitride fibers were systematically examined. As a result, a boron nitride fiber having a degree of orientation of less than 0.5 has substantially the same tensile strength as that of a boron nitride fiber whose C planes are not predominantly oriented in a direction parallel to the fiber axis. In contrast, a boron nitride fiber having a degree of orientation of 0.5 or above has a tensile strength significantly higher than that of a non-oriented boron nitride fiber. For example, both of boron nitride fibers having degrees of orientation of 0.26 and 0.46 had a tensile strength of 440 MPa, while a boron nitride fiber having a degree of orientation of 0.80 had a tensile strength of 1,970 MPa.

In boron nitride fibers having degrees of orientation of 0.7 or above, the tensile strength of fiber increases substantially in proportion to the degree of orientation of fiber under the same given condition. For example, a fiber having a degree of orientation of 0.70 had a tensile strength of 840 MPa, while a fiber having a degree of orientation of 0.78 had an increased tensile strength of 1,400 MPa. Thus, in a fiber having a degree of orientation of 0.70 or above, the tensile strength can be further increased by increasing the degree of orientation.

The boron nitride fiber of the present invention has a tensile strength of at least 1,400 MPa, preferably at least 1,660 MPa, more preferably at least 1,870 MPa, further preferably at least 1,890 MPa, furthermore preferably at least 1,910 MPa, particularly preferably at least 1,970 MPa, most preferably at least 2,300 MPa.

The above tensile strength can be measured in accordance with "Testing Methods for Carbon Fibers" specified by JIS R 7601 (1986).

The boron nitride fiber of the present invention has a degree of orientation of at least 0.74, preferably at least 0.78, more preferably at least 0.80, further preferably at least 0.81, furthermore preferably at least 0.82, particularly preferably at least 0.83, most preferably at least 0.86.

An increase in a degree of orientation increases not only tensile strength but also thermal conductivity in fiber axis direction. In the case of graphite single crystal, it is known that the thermal conductivity in the direction parallel to the plane formed by linkage between six-carbon-membered rings is higher than that in the direction perpendicular to the plane. Also, in the case of a carbon fiber in which the six-carbon-membered rings are predominantly oriented to a direction parallel to the fiber axis, it is known that an increase in degree of orientation gives an increased thermal conductivity.

Meanwhile, in the case of boron nitride, it is known that when a boron nitride obtained by piling up the C planes of boron nitride regularly by chemical vapor phase method is

measured for thermal conductivity, the thermal conductivity in the direction parallel to the C plane is about 100 times as high as that in the direction perpendicular to the C plane. Hence, it is thought that a boron nitride fiber of high degree of orientation, as compared with a boron nitride fiber of low degree of orientation, has a high thermal conductivity in the fiber axis direction. In general, boron nitride has a thermal conductivity about 10 times as high as those of alumina, mullite, silicon nitride, etc.; therefore, there are cases that the thermal conductivity of a material is increased by blending it with boron nitride to form a composite material. In such cases, the thermal conductivity of the composite material can be increased efficiently by the use of a boron nitride fiber with an improved degree of orientation because the fiber has an increased thermal conductivity in the direction of the fiber axis.

The above-mentioned degree of orientation can be measured, by X-ray diffractometry, based on the distribution of X-ray intensity on the Debye ring formed by X-ray diffraction from C planes of hexagonal or turbostratic boron nitride. The method for measurement of degree of orientation by X-ray diffractometry is described below.

Using, as an X-ray for diffractometry, a copper  $K\alpha$  ray monochromatised using a nickel filter (the copper  $K\alpha$  ray is hereinafter referred to as "Cu  $K\alpha$  ray"), diffraction intensity is measured by transmission method. The source for X-ray desirably has a circular cross section in order to obtain diffraction at a high efficiency from the X-ray output used.

A fiber bundle consisting of several tens to several hundreds of boron nitride fibers is fixed using, for example, a small amount of collodion, in such a manner that the boron nitride fibers are arranged as parallel as possible, and the resulting bundle is used as a sample to be subjected to X-ray diffraction. This sample is hereinafter referred to as "sample for X-ray diffraction".

The measurement of diffraction intensity can be conducted using any of a method of photographing a diffraction pattern and a method using an X-ray diffractometer.

In measurement of diffraction intensity by the method of photographing a diffraction pattern, a sample for X-ray diffraction is fixed so that the fiber axis of each boron nitride fiber of the sample for X-ray diffraction is in a plane perpendicular to an incident X-ray and that the X-ray can be applied, without fail, to the sample for X-ray diffraction, i.e. the boron nitride fibers bundle. At this time, the direction of the fiber axis of each fiber of the sample for X-ray diffraction, in a plane perpendicular to the incident X-ray may be any desired direction as long as its direction relative to the diffraction pattern formed can be known. Herein, however, the fiber axis is fixed vertically for explanation purpose.

An X-ray-sensitive film for photographing a diffraction pattern formed is placed at the side of the sample for X-ray diffraction, opposite to the sample side to which an X-ray is applied. The X-ray-sensitive film is placed perpendicularly to the direction of the incident X-ray. The distance from the sample for X-ray diffraction to the X-ray-sensitive film (the distance is hereinafter referred to as "camera length" in some cases) must be such as to allow photographing of the whole portion of a Debye ring formed by the diffraction from the C planes of the hexagonal or turbostratic boron nitride constituting each boron nitride fiber of the sample for X-ray diffraction. The radius (D) of Debye ring on X-ray-sensitive film is determined from the following formula (1):

$$D=L\tan(2\theta) \quad (1)$$

(wherein L is a camera length; and  $2\theta$  is an angle of diffraction from the C planes of the hexagonal or turbostratic

boron nitride constituting each boron nitride fiber of the sample for X-ray diffraction, which satisfies Bragg condition. In the case of the hexagonal or turbostratic boron nitride constituting each boron nitride fiber,  $2\theta$  is in the range of  $24^\circ$ – $26^\circ$  when the incident X-ray is a Cu  $K\alpha$  ray. Hence, the camera length L can be determined so that a circle of radius D having its center at an intersecting point of the direction of an incident X-ray and the X-ray-sensitive film, is contained in the X-ray-sensitive film.

10 Intensity of diffracted X-ray varies depending mainly upon the amount of boron nitride fiber in sample for X-ray diffraction, and upon the crystallite size of hexagonal or turbostratic boron nitride constituting the fiber, etc. Therefore, the exposure time of X-ray used must be controlled in order to obtain an optimum diffraction pattern. When the exposure time is too long, the blackening of X-ray-sensitive film by diffracted X-ray is not proportional to the intensity of diffracted X-ray; as a result, in the obtained distribution of intensity of diffracted X-ray, the portion of strong intensity is relatively weaker than actual, and no accurate degree of orientation can be obtained. When the exposure time is too short, the S/N ratio of blackening of X-ray-sensitive film by diffracted X-ray is small and the degree of orientation obtained has a large error. An appropriate exposure time can be determined by photographing various diffraction patterns of the same sample for X-ray diffraction in various exposure times and confirming that there is no change in the degree of orientations obtained.

By developing the X-ray-sensitive film after X-ray application, the X-ray-irradiated portion of the film blackens in proportion to the intensity of diffracted X-ray applied. Therefore, by measuring the blackening degree of the film using a microdensitometer, the intensity of diffracted X-ray applied can be determined. When the C planes of the hexagonal or boron nitride constituting each boron nitride fiber of the sample for X-ray diffraction are oriented parallel to the fiber axis direction of the boron nitride fiber, there appears, on the Debye ring formed on the X-ray-sensitive film, such a distribution of diffraction intensity that the blackening degree of the film is maximum in a direction passing the center of the Debye ring, i.e. an intersecting point between incident X-ray and X-ray-sensitive film and perpendicular to the fiber axis of each boron nitride fiber of the sample for X-ray diffraction (the direction is hereinafter referred to as "equator direction" in some cases) and that the blackening degree of the film is minimum in a direction passing the center of the Debye ring and parallel to the fiber axis of each boron nitride fiber of the sample for X-ray diffraction (the direction is hereinafter referred to as "meridian direction" in some cases). The position of each point on Debye ring to be measured for diffraction intensity is determined by a central angle  $\phi$  measured from an arbitrarily selected base point on Debye ring, and the intensity of diffracted X-ray of each measurement point on Debye ring is determined as a function of the central angle  $\phi$ . At this time, the intensity of diffracted X-ray on Debye ring is a sum of the intensity of X-ray diffracted from the C planes of each boron nitride fiber and the intensity of the background. Hence, in order to obtain a net intensity of X-ray diffracted from C planes, the change in X-ray intensity in the radial direction of Debye ring is measured to determine the background intensity on Debye ring and then the background intensity is subtracted from the intensity of diffracted X-ray on Debye ring. By determining the intensity of X-ray diffracted from C planes, as a function of central angle  $\phi$ , there can be obtained two peaks at positions corresponding to the equator direction. The full width at half maximum

## 11

(unit=degree) is measured for the each peak and the average (H) of the two widths is calculated. Using this H, degree of orientation ( $\pi$ ) of crystal can be calculated from the following formula (2) ["Development and Evaluation of Carbon Fibers", p. 118 (1989), compiled by The Carbon Society of Japan].

$$\pi = (180 - H)/180 \quad (2)$$

Diffraction intensity can also be measured by the use of an X-ray diffractometer. The diffractometer may be a known diffractometer, but description is hereinafter made on a diffractometer in which the diffractometer axis is vertical and the scanning plane of a detector is horizontal. When an X-ray diffractometer is used, a fiber sample holder is used which can fix a sample for X-ray diffraction and which has a mechanism capable of rotating the sample in the range of 360° in a plane perpendicular to an X-ray applied.

First, there is determined, by transmission method, an angle of diffraction at which the C planes of the hexagonal or turbostratic boron nitride constituting each boron nitride fiber of a sample for X-ray diffraction satisfy Bragg condition. The sample for X-ray diffraction is fixed to the fiber sample holder, and the fiber axis of each boron nitride fiber of the sample is fixed perpendicularly. In this state, an X-ray is applied to the sample and the detector, i.e. the 2θ of the diffractometer is scanned to measure the intensity of diffracted X-ray. Since the diffraction from the C planes of hexagonal or turbostratic boron nitride takes place generally at 2θ=24° to 26°, there is measured, in this angle range, an angle at which the intensity of diffracted X-ray becomes maximum. This angle is taken as "diffraction angle of C planes". Next, the detector is fixed to the diffraction angle of C planes; an X-ray is applied; and the sample for X-ray diffraction fixed to the fiber sample holder is rotated in the range of 360° in a plane perpendicular to the X-ray applied, to measure the intensities of diffracted X-ray. Now, the rotational angle of the sample for X-ray diffraction is taken as  $\alpha$  (unit: degree); and a state in which the fiber axis of each boron nitride fiber of the sample is vertical, is taken as  $\alpha=0^\circ$ . When the C planes of the hexagonal or turbostratic boron nitride constituting each boron nitride fiber of the sample are oriented in a direction of the fiber axis of each boron nitride fiber, the diffracted X-ray gives two intensity peaks at  $\alpha=0^\circ$  and  $\alpha=180^\circ$ . At this time, a net intensity of diffracted X-ray must be obtained by subtracting the intensity of background in the same manner as in the above-mentioned case of photographing a diffraction pattern. The full widths at half maximum (unit: degree) are measured for the two peaks and, using the average (H) of the widths obtained, a degree of orientation ( $\pi$ ) can be calculated from the formula (2).

There is no particular restriction for production of the boron nitride fiber of the present invention having a large tensile strength and C planes of high degree of orientation. However, the present boron nitride fiber can be typically produced as follows.

(a) First, a boron trihalide-nitrile compound adduct is reacted with an ammonium halide or a primary amine hydrohalide in the presence of a boron trihalide to form a boron nitride precursor.

The boron trihalide includes boron trifluoride, boron trichloride, boron tribromide, boron triiodide, etc. They can be used with no particular restriction.

As the nitrile compound, a known compound having a nitrile group can be used with no particular restriction. Specific examples of the nitrile compound are acetonitrile, propionitrile, capronitrile, acrylonitrile, crotononitrile, tolunitrile, benzonitrile, isobutyronitrile, n-butynitrile,

## 12

isovaleronitrile, 2-methylbutyronitrile, pivalonitrile, n-valeronitrile, malononitrile, succinonitrile, glutaronitrile, adiponitrile, pimelonitrile and suberonitrile. As the number of carbon atoms of the nitrile compound increases, the amount of carbon in the resulting boron nitride precursor increases and the amount of carbon to be eliminated becomes large in order to convert the boron nitride precursor to boron nitride by heat treatment. Therefore, use of a nitrile compound having a less amount of carbon atoms, such as acetonitrile, acrylonitrile or the like is preferred.

The ammonium halide includes ammonium fluoride, ammonium chloride, ammonium bromide, ammonium iodide, etc. A preferable example of the ammonium halide is ammonium chloride.

15 The primary amine hydrohalide includes a primary amine hydrofluoride, a primary amine hydrochloride, a primary amine hydrobromide, a primary amine hydroiodide, etc. A preferable example of the primary amine hydrohalide is a primary amine hydrochloride.

20 The primary amine hydrochloride is represented by a general formula  $RNH_2 \cdot HCl$ , and there can be used, with no restriction, a compound wherein R is an alkyl group such as methyl, ethyl, propyl or the like, or an aryl group such as phenyl, tolyl, xylyl or the like. However, use of a primary

25 amine hydrochloride wherein R is a lower alkyl group such as methyl, ethyl or the like, is preferred because as the number of carbon atoms of R increases, the amount of carbon in the resulting boron nitride precursor increases and the amount of carbon eliminated becomes large in order to 30 convert the boron nitride precursor to boron nitride by heat treatment.

In order to obtain the boron nitride fiber of the present invention, first, an adduct between the above-mentioned boron halide and nitrile compound is reacted with the 35 above-mentioned ammonium halide or primary amine hydrohalide to form a boron nitride precursor.

The adduct between the boron trihalide and the nitrile compound is a product wherein the boron of boron trihalide is bonded, by an addition reaction, to the non-bonded 40 electron pair of the nitrogen atom of the nitrile group. The boron trihalide and the nitrile compound react with each other easily to form the adduct. There is no particular restriction as to the method for forming the adduct. The adduct can be formed, for example, by a method which

45 comprises dissolving a nitrile compound in an organic solvent and adding a boron trihalide dropwise to the solution at room temperature, a method which comprises dissolving a nitrile compound in an organic solvent and introducing a gaseous boron trihalide into the solution by bubbling, or a 50 method which comprises dissolving a boron trihalide in an organic solvent and adding a nitrile compound dropwise to the solution. Since the boron trihalide and the nitrile compound react with each other easily to form an adduct, the two materials may be contacted right before the reaction.

55 At the time when the adduct is reacted with the ammonium halide or the primary amine hydrohalide, presence of a boron trihalide is essential. When no boron trihalide is present during the above reaction, the yield of the boron nitride precursor is low and a by-product is formed which is 60 insoluble in the solvent used in spinning (mentioned later), for example, N,N-dimethylformamide (hereinafter referred to as DMF, in some cases).

It is sufficient that the boron trihalide is present at least during the reaction of the boron trihalide-nitrile compound 65 adduct with the ammonium halide or the primary amine hydrohalide. For example, by using the boron trihalide in excess in forming the boron trihalide-nitrile compound

adduct, unreacted boron trihalide and the adduct may be allowed to coexist. The amount of the boron trihalide used relative to the nitrile compound can be selected as desired in the range of 1.05–2.00 in terms of boron trihalide/nitrile compound molar ratio. However, since too small an amount of the boron trihalide invites formation of DMF-insoluble compound and too large an amount of the boron trihalide gives an increased amount of the boron trihalide not contributing to the reaction, the boron trihalide/nitrile compound molar ratio is preferably 1.1–1.5. Since the boron trihalide and the nitrile compound form an adduct at a 1:1 molar ratio, the amount of the boron trihalide present during the reaction of the adduct with the ammonium halide or the primary amine hydrohalide is 0.1–0.5 in terms of boron trihalide/adduct molar ratio.

There is no particular restriction as to the concentration of the nitrile compound in the reaction solvent. The concentration, however, is preferably in the range of 0.1–10 mole/l. When the concentration of the nitrile compound is less than 0.1 mole/l, the amount of the resulting boron nitride precursor is small, which is inefficient and not desirable. When the concentration of the nitrile compound is more than 10 mole/l, the amount of the solid adduct formed is too large relative to the amount of the solvent and the homogeneous formation of the adduct is prevented, which is not desirable.

The amount of the ammonium halide or primary amine hydrohalide added is preferably selected in the range of 0.67–1.5 in terms of ammonium halide or primary amine hydrohalide/nitrile compound molar ratio. When the amount of the ammonium halide or primary amine hydrohalide is too large, a DMF-insoluble compound is formed. When the amount of the nitrile compound is too large, the amount of unreacted adduct tends to increase. Therefore, selection of the above molar ratio in the range of 0.83–1.2 is more preferable.

There is no particular restriction as to the solvent used for synthesis of the boron nitride precursor of the present invention. However, it is preferable that the solvent can easily dissolve and remove the reaction by-products such as borazine compound and the like in separating the reaction product, i.e. the boron nitride precursor. From this standpoint, there is preferably selected an organic solvent such as benzene, toluene, xylene, chlorobenzene or the like.

The reaction temperature employed for reacting the adduct with the ammonium halide or the primary amine hydrohalide is preferably selected in the range of 100°–160° C. because, in general, use of a low temperature requires a long reaction time and use of a high temperature produces an increased amount of by-products insoluble in DMF and gives a reduced yield. The reaction time is preferably selected in the range of 3–30 hours although it varies depending upon the reaction temperature employed.

The above heating treatment produces a boron nitride precursor in the form of an orange-colored or brown precipitate.

As the reactor for obtaining the boron nitride precursor, a known reactor is used with no particular restriction. However, since both the boron trihalide-nitrile compound adduct and the boron nitride precursor undergo hydrolysis, it is necessary that the reaction system inside is beforehand dried thoroughly with nitrogen gas or the like and that a moisture-absorbing agent such as calcium chloride or the like is provided at the open part of the reactor to prevent the incoming of moisture in air from outside the reaction system during the reaction.

(b) The boron nitride precursor produced in the above step (a) is dissolved in a solvent to prepare a boron nitride precursor solution.

The boron nitride precursor solution can be used as a spinning solution in the next step (c).

For preparing the boron nitride precursor fiber from the boron nitride precursor, a known method can be used with no particular restriction. For example, when the boron nitride precursor solution is spun to obtain a precursor fiber, the boron nitride precursor is dissolved in a precursor-soluble solvent to prepare a spinning solution. The precursor-soluble solvent includes, for example, DMF,  $\epsilon$ -caprolactam, crotononitrile, malonitrile, N-methyl- $\beta$ -cyanoethylformamide and N,N-diethylformamide. By dissolving the boron nitride precursor in the precursor-soluble solvent, an orange-colored or brown transparent spinning solution is obtained.

The viscosity of the spinning solution can as necessary be controlled, for example, by the addition of an acrylonitrile polymer. When the boron nitride precursor has a relatively small molecular weight, an acrylonitrile polymer having a relatively large molecular weight is used together with the precursor, whereby the resulting spinning solution can have a higher viscosity and improved spinnability.

There is no particular restriction as to the acrylonitrile polymer used in the present invention, as long as the polymer is soluble in the solvent constituting the spinning solution and causes no phase separation from the boron nitride precursor in the spinning solution. The acrylonitrile polymer is preferably a polymer of acrylonitrile or a copolymer of acrylonitrile and a vinyl group-containing polymerizable monomer other than acrylonitrile (the monomer is hereinafter referred to simply as "vinyl monomer"), such as vinyl acetate, acrylamide, methacrylic acid, methacrylic acid ester, acrylic acid, acrylic acid ester or the like. When an acrylonitrile/vinyl monomer copolymer is used, the proportion of acrylonitrile in the copolymer is preferably 85 mole % or more based on the total polymerizable monomers because an increase in amount of vinyl monomer in the copolymer tends to cause phase separation of the copolymer from the boron nitride precursor in the spinning solution. The vinyl monomer contains an oxygen atom(s), and the oxygen atom(s) may show adverse effects on the boron nitride fiber obtained, for example, growth of boron nitride crystals and consequent reduction in strength of boron nitride fiber. The acrylonitrile polymer, therefore, is more preferably an acrylonitrile homopolymer.

The weight-average molecular weight of the acrylonitrile polymer used in the present invention is not particularly restricted, but is preferably in the range of 10,000 to 2,000,000.

The amount of the acrylonitrile polymer added to the spinning solution is not particularly restricted, but is preferably 0.01–5 parts by weight per 100 parts by weight of the boron nitride precursor.

(c) The boron nitride precursor solution prepared in the step (b) is spun to form a boron nitride precursor fiber.

The preferable concentration range of the spinning solution is 0.01–3.0 g/ml although it varies depending upon the spinning method employed, and the viscosity employed during spinning is 10–100,000 poises. For spinning a boron nitride precursor fiber from the spinning solution, a well known method can be used. A boron nitride precursor fiber can be spun, for example, by a method of rotating a small-hole-provided vessel containing a spinning solution, to extrude the spinning solution from the hole by the utilization of a centrifugal force; a method of extruding a spinning solution from a small hole by the utilization of a gas pressure; or a method of extruding a spinning solution from a small hole by the utilization of a gear pump.

## 15

The spinning temperature is, for example, -60° to 200° C., preferably -10° to 180° C., more preferably 0° to 160° C. although it varies depending upon the solvent used.

- (d) The boron nitride precursor fiber is preheated at 100°-600° C. in an inert gas atmosphere.  
 (e) The preheated fiber is ammonia-treated at 200°-1,300° C. in an ammonia gas atmosphere.

That is, the boron nitride precursor fiber obtained in the step (c) is heat-treated (preheated) at 100°-600° C. in an inert gas atmosphere, and then heat-treated at 200°-1,300° C. in an ammonia gas atmosphere to obtain a boron nitride fiber. The boron nitride fiber at this state is hereinafter called "non-oriented boron nitride fiber". In producing the non-oriented boron nitride fiber, when only the heat treatment in an inert gas atmosphere is conducted, it is impossible to remove the carbon derived from the boron nitride precursor and the resulting fiber is black. When only the heat treatment in an ammonia gas atmosphere is conducted, the boron nitride crystallite of the resulting boron nitride fiber becomes coarse and the fiber surface has flaws and scars, making it impossible to obtain a boron nitride fiber of high strength.

As the atmosphere gas used in the heat treatment conducted in an inert gas atmosphere, there can be used nitrogen, argon, helium, etc. The temperature used in the heat treatment in an inert gas atmosphere can be selected as desired in the range of 100°-600° C., preferably 150°-550° C., more preferably 160°-500° C. When the heat treatment in an inert gas atmosphere is conducted at a temperature lower than 100° C., in the subsequent heat treatment conducted in an ammonia gas atmosphere, the boron nitride crystallite becomes coarse, the surface of the resulting fiber has flaws and scars, and the fiber has a reduced strength in some cases. When the heat treatment in an inert gas atmosphere is conducted at a temperature higher than 600° C., the carbon derived from the precursor is easily graphitized and it is difficult to remove the graphite in the subsequent heat treatment in an ammonia gas atmosphere.

The heating apparatus used for conducting the heat treatment of the boron nitride precursor fiber in an inert gas atmosphere may be an apparatus having a structure capable of controlling the inside atmosphere by a chamber, a tube or the like. A known heating apparatus such as electric furnace, gas furnace or the like can be used with no particular restriction.

As the method for heat treatment, there are a batch-wise method of heat-treating a certain amount of a boron nitride precursor fiber at once; and a continuous method of feeding a continuous boron nitride precursor fiber continuously into a heating apparatus beforehand heated to a heat treatment temperature, to conduct a heat treatment and winding up the heat-treated fiber. Any of these heat treatment methods may be used in the present invention. When a batch-wise heat treatment is conducted in an inert gas atmosphere, it can be conducted by introducing a boron nitride precursor fiber into a heating apparatus beforehand heated to a heat treatment temperature, or by arranging a boron nitride precursor fiber in a heating apparatus and then heating the fiber to a heat treatment temperature.

In any of the above heat treatment methods, when the boron nitride precursor fiber is heated rapidly, the solvent (e.g. DMF) used in preparation of the spinning solution from the boron nitride precursor vaporizes rapidly or the separation of thermal decomposition products takes place rapidly, and the resulting boron nitride fiber has flaws such as voids, cracks and the like and has a reduced strength in some cases. It is therefore preferable that the heat treatment in an inert gas atmosphere is conducted by employing a temperature

## 16

elevation rate of 20° C./min or less up to the moment when the boron nitride precursor fiber reaches the heat treatment temperature. The retention time at the heat treatment temperature can be selected as desired in the range of 0-10 hours. A retention time of 0 hour indicates that the heat treatment is terminated immediately after the boron nitride precursor fiber has reached the heat treatment temperature, for example, by cooling the heating apparatus or by taking the boron nitride precursor fiber out of the heating apparatus.

The atmosphere used in the heat treatment in an inert gas atmosphere is preferably an inert gas atmosphere in any of the temperature elevation step in which the boron nitride precursor fiber reaches the heat treatment temperature, the retention step in which the precursor fiber is retained at the heat treatment temperature, and the cooling step up to the completion of the heat treatment, that is, while the boron nitride precursor fiber is in the chamber, tube or the like of the heating apparatus containing the inert gas atmosphere. The inert gas atmosphere can be obtained by purging the chamber, tube or the like of the heating apparatus with an inert gas and then sealing the heating apparatus, or by passing an inert gas through the chamber, tube or the like of the heating apparatus.

Following the heat treatment in an inert gas atmosphere, a heat treatment in an ammonia gas atmosphere is conducted. The temperature employed in the heat treatment in an ammonia gas atmosphere can be selected as desired in the range of 200°-1,300° C. When the heat treatment in an ammonia gas atmosphere is conducted at a temperature lower than 200° C., the carbon derived from the precursor cannot be removed sufficiently and 5-15% by weight of carbon remains in the resulting boron nitride fiber. Since the carbon derived from the precursor is decomposed and removed almost completely by a heat treatment at 200°-1,300° C., preferably at 250°-1,250° C., more preferably at 300°-1,200° C., it is not necessary to conduct the heat treatment in an ammonia gas atmosphere, at a temperature higher than 1,300° C.

The heating apparatus used for conducting the heat treatment of the boron nitride precursor fiber in an ammonia gas atmosphere may be an apparatus having a structure capable of controlling the inside atmosphere by a chamber, a tube or the like. A known heating apparatus such as electric furnace, gas furnace or the like can be used with no particular restriction. The method used for conducting the heat treatment may be any of a batch-wise method and a continuous method as in the case of the heat treatment in an inert gas atmosphere. When a batch-wise heat treatment is conducted, it is conducted by introducing a boron nitride precursor fiber into a heating apparatus heated beforehand to a heat treatment temperature, or by arranging a boron nitride precursor fiber in a heating apparatus and then heating the fiber to a heat treatment temperature.

In any of the above heat treatment methods, when the boron nitride precursor fiber is heated rapidly, the separation of thermal decomposition products takes place rapidly and the resulting boron nitride fiber has flaws such as voids, cracks and the like and has a reduced strength in some cases. It is therefore preferable that the heat treatment is conducted by employing a temperature elevation rate of 20° C./min or less up to the moment when the boron nitride precursor fiber reaches the heat treatment temperature. The retention time at the heat treatment temperature can be selected as desired in the range of 0-10 hours although it varies depending upon the amount of the boron nitride precursor fiber to be heat-treated. A retention time of 0 hour indicates that the heat treatment is terminated immediately after the boron nitride

precursor fiber has reached the heat treatment temperature, by cooling the heating apparatus or by taking the boron nitride precursor fiber out of the heating apparatus.

In the heat treatment in an ammonia gas atmosphere, an ammonia gas atmosphere must be used in the temperature elevation step from the temperature of heat treatment in an inert gas atmosphere to the temperature of heat treatment in an ammonia gas atmosphere, and in the retention step at the temperature of heat treatment in an ammonia gas atmosphere. In other heat treatment steps, i.e. the temperature elevation step up to the temperature of heat treatment in an inert gas atmosphere and the cooling step from the temperature of heat treatment in an ammonia gas atmosphere, it is possible to use any of an inert gas atmosphere (e.g. nitrogen, argon or helium) and an ammonia gas atmosphere. The ammonia gas atmosphere can be obtained by purging the chamber, tube or the like of the heating apparatus with an ammonia gas and then sealing the heating apparatus, or by passing an ammonia gas through the chamber, tube or the like of the heating apparatus.

In the present invention, it is preferable that first a heat treatment (preheating) is conducted in an inert gas atmosphere and then a heat treatment is conducted in an ammonia gas atmosphere. The heat treatment in an inert gas atmosphere and the heat treatment in an ammonia gas atmosphere in this order may be carried out by first conducting the heat treatment in an inert gas atmosphere and, when the heat treatment is over, switching the atmosphere gas to ammonia to successively conduct the heat treatment in an ammonia gas atmosphere, or by completing the heat treatment in an inert gas atmosphere by cooling the heating apparatus or by taking the resulting boron nitride fiber out of the heating apparatus, and then newly conducting the heat treatment in an ammonia gas atmosphere.

(f) The ammonia-treated fiber obtained in the step (e) is heated at 1,600°–2,300° C. in an inert gas atmosphere with a tensile stress being applied to the fiber, whereby a boron nitride fiber of the present invention is obtained.

That is, a boron nitride fiber having a degree of orientation of 0.74 or above can be obtained by heat-treating a non-oriented boron nitride fiber at 1,600°–2,300° C., preferably at 1,650°–2,250° C., more preferably at 1,700°–2,200° C. in an inert gas atmosphere with a tensile stress being applied to the fiber (the heat treatment is hereinafter referred to as "orientation treatment" in some cases).

There is no particular restriction for the atmosphere used in the orientation treatment as long as the boron nitride of the non-oriented boron nitride fiber undergoes no chemical change caused by oxidation, etc. The atmosphere gas used in the orientation treatment may therefore be an inert gas such as nitrogen, argon, helium or the like. The orientation treatment may also be conducted in vacuum.

The temperature used in the orientation treatment can be selected as desired in the range of 1,600°–2,300° C. When the temperature is lower than 1,600° C., orientation does not proceed sufficiently even with a tensile stress applied and the resulting degree of orientation does not reach 0.74 in some cases. When the temperature is 2,300° C. or higher, the decomposition of boron nitride begins; therefore, the orientation treatment at 2,300° C. or higher is not preferable.

The heating apparatus used for conducting the orientation treatment may be an apparatus having a structure capable of controlling the inside atmosphere by a chamber, a tube or the like. A known heating apparatus such as electric furnace, gas furnace or the like can be used with no particular restriction. As the method for orientation treatment, there are a batch-wise method of treating a certain amount of a non-oriented

boron nitride fiber at once; and a continuous method of feeding a continuous non-oriented boron nitride fiber continuously into a heating apparatus heated beforehand to an orientation treatment temperature, to conduct an orientation treatment and winding up the oriented fiber. Any of these orientation treatment methods may be used in the present invention. When a batch-wise orientation treatment is conducted, it can be conducted by introducing a non-oriented boron nitride fiber into a heating apparatus heated beforehand to an orientation treatment temperature, or by arranging a non-oriented boron nitride fiber in a heating apparatus and then heating the fiber to an orientation treatment temperature.

In the orientation treatment, when the non-oriented boron nitride fiber is heated rapidly, the resulting boron nitride fiber has flaws caused by the thermal stress applied and has a reduced strength in some cases. It is therefore preferable that the orientation treatment is conducted by employing a temperature elevation rate of 100° C./min or less up to the moment when the non-oriented boron nitride fiber reaches the orientation treatment temperature. The retention time at the orientation treatment temperature can be selected as desired in the range of 0–10 hours although it varies depending upon the amount and orientation treatment temperature of the non-oriented boron nitride fiber to be subjected to an orientation treatment. A retention time of 0 hour indicates that the orientation treatment is terminated immediately after the non-oriented boron nitride fiber has reached the orientation treatment temperature, by cooling the heating apparatus or by taking the non-oriented boron nitride fiber out of the heating apparatus.

The atmosphere used in the orientation treatment is preferably an inert gas atmosphere or vacuum in any of the temperature elevation step in which the non-oriented boron nitride fiber reaches the orientation treatment temperature, the retention step in which the non-oriented fiber is retained at the orientation treatment temperature, and the cooling step up to the completion of the orientation treatment. The inert gas atmosphere can be obtained by purging the chamber, tube or the like of the heating apparatus with an inert gas and then sealing the heating apparatus, or by passing an inert gas through the chamber, tube or the like of the heating apparatus.

There is no particular restriction as to the method for applying a tensile stress to the non-oriented boron nitride fiber in the orientation treatment. For example, when the orientation treatment is conducted batch-wise, the application of tensile stress can be conducted by suspending a non-oriented boron nitride fiber vertically and adding a weight to the lower end of the fiber. Alternatively, when a non-oriented boron nitride fiber is heat-treated at 1,600°–2,300° C. in an inert gas with no tensile stress applied, the fiber causes shrinkage in the fiber axis direction depending upon the heat treatment temperature; therefore, when a non-oriented boron nitride fiber is wound round a frame made of a material (e.g. boron nitride) not reactive with the fiber and is heat-treated in that state at 1,600°–2,300° C. in an inert gas atmosphere, the thermal shrinkage of the non-oriented boron nitride fiber caused by the heat treatment is prevented by the presence of the frame, which is essentially the same as the heat treatment of the non-oriented boron nitride fiber under application of a tensile stress. When the orientation treatment is conducted continuously, the thermal shrinkage of a non-oriented boron nitride fiber in the heat treatment can be controlled by controlling the rate of feeding of the fiber to a heating apparatus and the winding-up rate of the fiber after the heat treatment; as a result, the heat treatment (orientation treatment) can be conducted with a tensile stress being applied.

The tensile stress applied to a non-oriented boron nitride fiber in the orientation treatment varies depending upon the temperature and time of the orientation treatment, but can be selected as desired in the range of 0.1-1,000 MPa when a stress is applied, for example, by using a weight. When the stress applied is smaller than 0.1 MPa, orientation takes place insufficiently and the resulting degree of orientation does not reach 0.74 in some cases. When the stress applied is larger than 1,000 MPa, the non-oriented fiber breaks in some cases. Meanwhile, when a tensile stress is applied to a non-oriented boron nitride fiber by restricting the thermal shrinkage of the fiber caused by the heat treatment, or, in the case of the continuous orientation treatment, controlling the rate of feeding of the fiber to a heating apparatus and the winding-up rate of the fiber after the heat treatment to restrict the thermal shrinkage of the fiber caused by the heat treatment, the elongation ratio can be selected in the range of, for example, 10-32%. Herein, the elongation ratio (E) is defined by the following formula (3):

$$E=100 \times (L_s - L_f) / L_s \quad (3)$$

wherein  $L_s$  represents a fiber length when a boron nitride fiber sample of unit length has been heat-treated at a temperature ( $T$  °C.) without restricting the thermal shrinkage of the sample, in other words, without applying any tensile stress to the sample; and  $L_f$  represents a fiber length when the same boron nitride fiber sample of unit length has been heat-treated at the same temperature ( $T$  °C.) while restricting the thermal shrinkage of the sample.

When the elongation ratio is smaller than 10%, the tensile stress applied to the non-oriented boron nitride fiber is insufficient and the resulting degree of orientation does not reach 0.74 in some cases. When the elongation ratio is larger than 32%, the non-oriented boron nitride fiber breaks during the orientation treatment in some cases.

The oriented boron nitride fiber produced as above has features that the crystallite size of boron nitride constituting the fiber are very small and that the fiber is white and has luster.

For production of the boron nitride fiber of the present invention, there is, for example, a process which comprises reacting an adduct between boron trichloride and a nitrile compound having 3 or less carbon atoms with ammonium chloride in the presence of boron trichloride to form a boron nitride precursor, dissolving the precursor in N,N-dimethylformamide (a solvent), spinning the resulting solution to form a precursor fiber, heat-treating the precursor fiber at 100°-600° C. in an inert gas atmosphere and then at 600°-1,300° C. in an ammonia gas atmosphere to form a boron nitride fiber, and heat-treating the fiber at 1,600°-2,300° C. with a tensile stress being applied. This process is preferable because it produces a boron nitride fiber at a high yield, the amount of residual carbon in the boron nitride fiber is reduced to be negligible, and the process operation is easy.

#### Industrial Applicability

The present invention allows production of a boron nitride fiber composed mainly of hexagonal and/or turbostratic boron nitride having C planes oriented parallel to the fiber axis and a degree of orientation of 0.74 or above. As a result, a boron nitride fiber having a remarkably increased tensile strength can be produced, and it has become possible to produce a boron nitride fiber having not only the heat resistance, oxidation resistance, solid lubricity and low reactivity inherently possessed by boron nitride, but also a high strength. Accordingly, the boron nitride fiber of the present invention can be applied as an excellent reinforcing fiber used for improvement of the toughness of ceramic material or the like to obtain a composite material.

#### EXAMPLES

The present invention is hereinafter described in detail by way of Examples. However, the present invention is in no way restricted to these Examples.

The tensile strength of a fiber is greatly influenced by the degree of orientation of the C planes of the fiber, but tends to be affected by the flaws, scars, etc. of the fiber surface which vary depending upon the spinning method employed.

10 In the present invention, therefore, the change in tensile strength brought about by the change in degree of orientation in various fibers produced under the same conditions has an important meaning.

In the Examples, the yield of each boron nitride fiber precursor was determined based on the amount of boron (B) in the boron trihalide used as a starting material.

Each boron nitride fiber obtained in Examples and Comparative Examples was identified by confirming that it showed an absorption of BN at around  $1,380 \text{ cm}^{-1}$  and around  $800 \text{ cm}^{-1}$  in IR absorption spectrum and that it showed the maximum signal at around  $20=26^\circ$  in powder X-ray diffractometry.

#### Example 1

25 In a three-necked flask having a capacity of 1 l, the center tube was provided with a stirrer; one of the side tubes was provided with a Dewar type cold finger to which a boron trichloride-containing cylinder was connected; and the remaining side tube was provided with an Allihn condenser. To the Allihn condenser was fitted a Dewar type cold finger, and a calcium chloride tube was fitted to the outlet of the cold finger. Through the resulting apparatus was passed dry nitrogen at a rate of 200 ml/min for 4 hours to dry the apparatus inside. In the apparatus were placed 16.4 g of acetonitrile and 300 ml of chlorobenzene which had been dried overnight with anhydrous sodium sulfate. The two cold fingers were filled with dry ice-acetone. Boron trichloride of 60 g was added dropwise for 2 hours from a cold finger fitted directly to the three-necked flask to the contents of the flask which were stirred with the stirrer. Thereby, a white boron trichloride-acetonitrile adduct was formed. After the completion of the dropwise addition of boron trichloride, the cold finger directly fitted to the three-necked flask was detached, and 21.5 g of ammonium chloride dried at 110° C. overnight was added. When the resulting suspension was heated at 125° C. for 8 hours, the generation of hydrogen chloride stopped substantially and a brown precipitate was formed. The precipitate was collected by filtration, washed with 100 ml of chlorobenzene, and dried under vacuum to obtain 24 g (yield: 83%) of a boron nitride precursor.

30 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 946

perature elevation from room temperature to 1,000° C. at a rate of 2° C./min in an ammonia gas atmosphere, then cooled to 500° C. at a rate of 5° C./min, and allowed to cool to room temperature, whereby a heat treatment was conducted. As a result, a non-oriented boron nitride fiber having a diameter of about 15  $\mu$ m was obtained.

The non-oriented boron nitride fiber was wound up in a loop shape having a circumference of 122 mm and, with the shape being retained, put round a boron nitride-made frame having a circumference of 103 mm. The fiber put round the frame was subjected to temperature elevation from room temperature to 1,800° C. at a rate of 10° C./min in a nitrogen current, kept at 1,800° C. for 30 minutes, cooled to 500° C. at a rate of 5° C./min, and allowed to cool to room temperature, whereby an orientation treatment was conducted. The boron nitride fiber after the treatment neither broke nor got loose, and retained a state of being wound round the frame. The elongation ratio after the orientation treatment was 12.7%. The boron nitride fiber obtained had a degree of orientation of 0.78 and a tensile strength of 1,400 MPa.

An X-ray (Cu K $\mu$ , 50 kV, 24 mA) was applied to the above boron nitride fiber from a direction perpendicular to the fiber axis. The resulting diffraction pattern was photographed. The photograph is shown in FIG. 1.

The above boron nitride fiber was also measured for IR absorption spectrum (KBr). The spectrum is shown in FIG. 3.

#### Example 2

The non-oriented boron nitride fiber produced in the same manner as in Example 1 was wound up in a loop shape having a circumference of 122 mm and, with the shape being retained, put round a boron nitride-made frame having a circumference of 103 mm. The fiber put round the frame was subjected to temperature elevation from room temperature to 2,000° C. at a rate of 10° C./min in a nitrogen current, kept at 2,000° C. for 30 minutes, cooled to 500° C. at a rate of 5° C./min, and allowed to cool to room temperature, whereby an orientation treatment was conducted. The boron nitride fiber after the treatment neither broke nor got loose, and retained a state of being wound round the frame. The elongation ratio after the orientation treatment was 15.7%. The boron nitride fiber obtained had a degree of orientation of 0.74 and a tensile strength of 1,660 MPa.

#### Example 3

The non-oriented boron nitride fiber produced in the same manner as in Example 1 was wound up in a loop shape having a circumference of 122 mm and, with the shape being retained, put round a boron nitride-made frame having a circumference of 107 mm. The fiber put round the frame was subjected to temperature elevation from room temperature to 2,000° C. at a rate of 10° C./min in a nitrogen current, kept at 2,000° C. for 30 minutes, cooled to 500° C. at a rate of 5° C./min, and allowed to cool to room temperature, whereby an orientation treatment was conducted. The boron nitride fiber after the treatment neither broke nor got loose, and retained a state of being wound round the frame. The elongation ratio after the orientation treatment was 20.2%. The boron nitride fiber obtained had a degree of orientation of 0.80 and a tensile strength of 1,970 MPa.

#### Example 4

The non-oriented boron nitride fiber produced in the same manner as in Example 1 was wound up in a loop shape

having a circumference of 122 mm and, with the shape being retained, put round a boron nitride-made frame having a circumference of 111 mm. The fiber put round the frame was subjected to temperature elevation from room temperature to 2,000° C. at a rate of 10° C./min in a nitrogen current, kept at 2,000° C. for 30 minutes, cooled to 500° C. at a rate of 5° C./min, and allowed to cool to room temperature, whereby an orientation treatment was conducted. The boron nitride fiber after the treatment neither broke nor got loose, and retained a state of being wound round the frame. The elongation ratio after the orientation treatment was 24.7%. The boron nitride fiber obtained had a degree of orientation of 0.86 and a tensile strength of 2,300 MPa.

#### Comparative Example 1

The non-oriented boron nitride fiber produced in the same manner as in Example 1 was wound up in a loop shape having a circumference of 122 mm and, with the shape being retained, put round a boron nitride-made frame having a circumference of 95 mm. The fiber put round the frame was subjected to temperature elevation from room temperature to 2,000° C. at a rate of 10° C./min in a nitrogen current, kept at 2,000° C. for 30 minutes, cooled to 500° C. at a rate of 5° C./min, and allowed to cool to room temperature, whereby an orientation treatment was conducted. The boron nitride fiber after the treatment neither broke nor got loose, and retained a state of being wound round the frame. The elongation ratio after the orientation treatment was 6.7%. The boron nitride fiber obtained had a degree of orientation of 0.66 and a tensile strength of 1,000 MPa.

#### Comparative Example 2

The non-oriented boron nitride fiber produced in the same manner as in Example 1 was wound up in a loop shape having a circumference of 122 mm and, with the shape being retained, put round a boron nitride-made frame having a circumference of 98 mm. The fiber put round the frame was subjected to temperature elevation from room temperature to 1,800° C. at a rate of 10° C./min in a nitrogen current, kept at 1,800° C. for 30 minutes, cooled to 500° C. at a rate of 5° C./min, and allowed to cool to room temperature, whereby an orientation treatment was conducted. The boron nitride fiber after the treatment neither broke nor got loose, and retained a state of being wound round the frame. The elongation ratio after the orientation treatment was 7.1%. The boron nitride fiber obtained had a degree of orientation of 0.70 and a tensile strength of 840 MPa.

#### Comparative Example 3

The non-oriented boron nitride fiber produced in the same manner as in Example 1 was wound up in a loop shape having a circumference of 122 mm and, with the shape being retained, put round a boron nitride-made frame having a circumference of 98 mm. The fiber put round the frame was subjected to temperature elevation from room temperature to 1,600° C. at a rate of 10° C./min in a nitrogen current, kept at 1,600° C. for 30 minutes, cooled to 500° C. at a rate of 5° C./min, and allowed to cool to room temperature, whereby an orientation treatment was conducted. The boron nitride fiber after the treatment neither broke nor got loose, and retained a state of being wound round the frame. The elongation ratio after the orientation treatment was 3.3%. The boron nitride fiber obtained had a degree of orientation of 0.46 and a tensile strength of 440 MPa.

#### Comparative Example 4

With no tensile stress applied, the non-oriented boron nitride fiber produced in the same manner as in Example 1

## 23

was subjected to temperature elevation from room temperature to 1,800° C. at a rate of 10° C./min in a nitrogen current, kept at 1,800° C. for 30 minutes, cooled to 500° C. at a rate of 5° C./min, and allowed to cool to room temperature, whereby an orientation treatment was conducted. The boron nitride fiber obtained had a degree of orientation of 0.35 and a tensile strength of 450 MPa.

An X-ray (Cu K $\mu$ , 50 kV, 24 mA) was applied to the above boron nitride fiber from a direction perpendicular to the fiber axis. The resulting diffraction pattern was photographed. The photograph is shown in FIG. 2.

## Comparative Example 5

With no tensile stress applied, the non-oriented boron nitride fiber produced in the same manner as in Example 1 was subjected to temperature elevation from room temperature to 1,600° C. at a rate of 10° C./min in a nitrogen current, kept at 1,600° C. for 30 minutes, cooled to 500° C. at a rate of 5° C./min, and allowed to cool to room temperature, whereby an orientation treatment was conducted. The boron nitride fiber obtained had a degree of orientation of 0.26 and a tensile strength of 440 MPa.

## Comparative Example 6

With no tensile stress applied, the non-oriented boron nitride fiber produced in the same manner as in Example 1 was subjected to temperature elevation from room temperature to 2,000° C. at a rate of 10° C./min in a nitrogen current, kept at 2,000° C. for 30 minutes, cooled to 500° C. at a rate of 5° C./min, and allowed to cool to room temperature, whereby an orientation treatment was conducted. The boron nitride fiber obtained had a degree of orientation of 0.37 and a tensile strength of 470 MPa.

## Example 5

The boron nitride precursor fiber produced in the same manner as in Example 1 was subjected to temperature elevation from room temperature to 400° C. at a rate of 1° C./min in a nitrogen current and then allowed to cool to room temperature, whereby a heat treatment was conducted. The resulting fiber was subjected to temperature elevation from room temperature to 400° C. at a rate of 2° C./min in an ammonia gas atmosphere and then allowed to cool to room temperature, whereby a heat treatment was conducted. Thereby, a non-oriented boron nitride fiber was obtained.

The non-oriented boron nitride fiber was subjected to an orientation treatment in the same manner as in Example 3. The elongation ratio after the orientation treatment was 20.2%. The boron nitride fiber obtained had a degree of orientation of 0.82 and a tensile strength of 1,930 MPa.

## Example 6

The boron nitride precursor fiber produced in the same manner as in Example 1 was subjected to temperature elevation from room temperature to 400° C. at a rate of 1° C./min in a nitrogen current and then allowed to cool to room temperature, whereby a heat treatment was conducted. The resulting fiber was subjected to temperature elevation from room temperature to 800° C. at a rate of 2° C./min in an ammonia gas atmosphere, then cooled to 500° C. at a rate of 5° C./min, and allowed to cool to room temperature, whereby a heat treatment was conducted. Thereby, a non-oriented boron nitride fiber was obtained.

The non-oriented boron nitride fiber was subjected to an orientation treatment in the same manner as in Example 3.

## 24

The elongation ratio after the orientation treatment was 20.3%. The boron nitride fiber obtained had a degree of orientation of 0.83 and a tensile strength of 1,910 MPa.

## Example 7

The boron nitride precursor fiber produced in the same manner as in Example 1 was subjected to temperature elevation from room temperature to 400° C. at a rate of 1° C./min in a nitrogen current and then allowed to cool to room temperature, whereby a heat treatment was conducted. The resulting fiber was subjected to temperature elevation from room temperature to 1,200° C. at a rate of 2° C./min in an ammonia gas atmosphere, then cooled to 500° C. at a rate of 5° C./min, and allowed to cool to room temperature, whereby a heat treatment was conducted. Thereby, a non-oriented boron nitride fiber was obtained.

The non-oriented boron nitride fiber was subjected to an orientation treatment in the same manner as in Example 3. The elongation ratio after the orientation treatment was 20.1%. The boron nitride fiber obtained had a degree of orientation of 0.82 and a tensile strength of 1,880 MPa.

## Example 8

25 The boron nitride precursor fiber produced in the same manner as in Example 1 was subjected to temperature elevation from room temperature to 200° C. at a rate of 1° C./min in a nitrogen current and then allowed to cool to room temperature, whereby a heat treatment was conducted. 30 The resulting fiber was subjected to temperature elevation from room temperature to 1,000° C. at a rate of 2° C./min in an ammonia gas atmosphere, then cooled to 500° C. at a rate of 5° C./min, and allowed to cool to room temperature, whereby a heat treatment was conducted. Thereby, a non-oriented boron nitride fiber was obtained.

The non-oriented boron nitride fiber was subjected to an orientation treatment in the same manner as in Example 3. The elongation ratio after the orientation treatment was 20.2%. The boron nitride fiber obtained had a degree of orientation of 0.82 and a tensile strength of 1,890 MPa.

## Example 9

In a three-necked flask having a capacity of 1 l, the center tube was provided with a stirrer; one of the side tubes was provided with a dropping funnel containing 128 g of boron tribromide; and the remaining side tube was provided with an Allihn condenser. To the outlet of the Allihn condenser was fitted a calcium chloride tube. Through the resulting apparatus was passed dry nitrogen at a rate of 200 ml/min for 4 hours to dry the apparatus inside. In the apparatus were placed 16.4 g of acetonitrile and 300 ml of chlorobenzene which had been dried overnight with anhydrous sodium sulfate. Into the apparatus contents being stirred with the stirrer was dropwise added, in 2 hours, boron tribromide from the dropping funnel. Thereby, a white boron tribromide-acetonitrile adduct was formed. After the completion of the dropwise addition of boron tribromide, the dropping funnel fitted to the three-necked flask was detached, and 21.5 g of ammonium chloride dried at 110° C. overnight was added. The resulting suspension was heated at 125° C. for 8 hours and then filtered. The precipitate collected was washed with 100 ml of chlorobenzene and dried under vacuum to obtain 48 g (yield: 80%) of a brown precipitate.

15 g of this boron nitride precursor was dissolved in 200 ml of DMF. 100 ml of the DMF was removed from the

## 25

resulting solution by vaporization, to obtain a uniform viscous solution. The solution was discharged into dry air at 25° C. from a spinning nozzle having holes of 60  $\mu\text{m}$  in diameter, by applying a back pressure of 15  $\text{kg}/\text{cm}^2$ , followed by winding-up, to obtain a continuous boron nitride precursor fiber having a diameter of about 20  $\mu\text{m}$ . At this time, the spinning solution had a viscosity of  $2.8 \times 10^4$  poises and the spinning speed was 1.9 m/min.

The boron nitride precursor fiber obtained above was heat-treated in the same manner as in Example 1, at 400° C. in a nitrogen current and then at 1,000° C. in an ammonia gas atmosphere, whereby a non-oriented boron nitride fiber having a diameter of about 15  $\mu\text{m}$  was obtained.

The non-oriented boron nitride fiber was subjected to an orientation treatment in the same manner as in Example 3. The elongation ratio after the orientation treatment was 20.2%. The boron nitride fiber obtained had a degree of orientation of 0.81 and a tensile strength of 1.870 MPa.

## Example 10

In a three-necked flask having a capacity of 1 l, the center tube was provided with a stirrer; one of the side tubes was provided with a dropping funnel containing 16.4 g of acetonitrile; and the remaining side tube was provided with an Allihn condenser. To the outlet of the Allihn condenser was fitted a calcium chloride tube. Through the resulting apparatus was passed dry nitrogen at a rate of 200 ml/min for 4 hours to dry the apparatus inside. In the apparatus were placed 200 g of boron triiodide and 300 ml of chlorobenzene which had been dried overnight with anhydrous sodium sulfate. Into the apparatus contents being stirred with the stirrer was dropwise added, in 2 hours, acetonitrile from the dropping funnel. Thereby, a white boron triiodide-acetonitrile adduct was formed. After the completion of the dropwise addition of boron triiodide, the dropping funnel fitted to the three-necked flask was detached, and 21.5 g of ammonium chloride dried at 110° C. overnight was added. The resulting suspension was heated at 125° C. for 8 hours and then filtered. The precipitate collected was washed with 100 ml of chlorobenzene and dried under vacuum to obtain 65 g (yield: 79%) of a brown precipitate.

20 g of this boron nitride precursor was dissolved in 200 ml of DMF. 100 ml of the DMF was removed from the resulting solution by vaporization, to obtain a uniform viscous solution. The solution was discharged into dry air at 25° C. from a spinning nozzle having holes of 60  $\mu\text{m}$  in diameter, by applying a back pressure of 15  $\text{kg}/\text{cm}^2$ , followed by winding-up, to obtain a continuous boron nitride precursor fiber having a diameter of about 20  $\mu\text{m}$ . At this time, the spinning solution had a viscosity of  $3.1 \times 10^4$  poises and the spinning speed was 1.7 m/min.

The boron nitride precursor fiber obtained above was heat-treated in the same manner as in Example 1, at 400° C. in a nitrogen current and then at 1,000° C. in an ammonia gas atmosphere, whereby a non-oriented boron nitride fiber having a diameter of about 15  $\mu\text{m}$  was obtained.

The non-oriented boron nitride fiber was subjected to an orientation treatment in the same manner as in Example 3. The elongation ratio after the orientation treatment was 20.1%. The boron nitride fiber obtained had a degree of orientation of 0.81 and a tensile strength of 1.880 MPa.

## Example 11

In a three-necked flask having a capacity of 1 l, the center tube was provided with a stirrer; one of the side tubes was

## 26

provided with a Dewar type cold finger to which a boron trichloride-containing bomb was connected; and the remaining side tube was provided with an Allihn condenser. To the Allihn condenser was fitted a Dewar type cold finger, and a calcium chloride tube was fitted to the outlet of the cold finger. Through the resulting apparatus was passed dry nitrogen at a rate of 200 ml/min for 4 hours to dry the apparatus inside. In the apparatus were placed 16.4 g of acetonitrile and 300 ml of chlorobenzene which had been dried overnight with anhydrous sodium sulfate. The two cold fingers were filled with dry ice-acetone. Into the apparatus contents being stirred with the stirrer was dropwise added, in 2 hours, 60 g of condensed boron trichloride from a cold finger fitted directly to the three-necked flask. Thereby, a white boron trichloride-acetonitrile adduct was formed. After the completion of the dropwise addition of boron trichloride, the cold finger directly fitted to the three-necked flask was detached, and 27.2 g of monomethylamine hydrochloride dried at 110° C. overnight was added. When the resulting suspension was heated at 125° C. for 8 hours, the generation of hydrogen chloride stopped substantially and a brown precipitate was formed. The precipitate was collected by filtration, washed with 100 ml of chlorobenzene, and dried under vacuum to obtain 25 g (yield: 80%) of a boron nitride precursor.

10 g of the boron nitride precursor was dissolved in 200 ml of DMF. 100 ml of the DMF was removed from the resulting solution by vaporization, to obtain a uniform viscous solution. The solution was discharged into dry air at 25° C. from a spinning nozzle having holes of 60  $\mu\text{m}$  in diameter, by applying a back pressure of 15  $\text{kg}/\text{cm}^2$ , followed by winding-up, to obtain a continuous boron nitride precursor fiber having a diameter of about 20  $\mu\text{m}$ . At this time, the spinning solution had a viscosity of  $3.0 \times 10^4$  poises and the spinning speed was 1.7 m/min.

The boron nitride precursor fiber obtained above was heat-treated in the same manner as in Example 1, at 400° C. in a nitrogen current and then at 1,000° C. in an ammonia gas atmosphere, whereby a non-oriented boron nitride fiber having a diameter of about 15  $\mu\text{m}$  was obtained.

15 The non-oriented boron nitride fiber was subjected to an orientation treatment in the same manner as in Example 3. The elongation ratio after the orientation treatment was 20.2%. The boron nitride fiber obtained had a degree of orientation of 0.82 and a tensile strength of 1.900 MPa.

## Example 12

In a three-necked flask having a capacity of 1 l, the center tube was provided with a stirrer; one of the side tubes was provided with a Dewar type cold finger to which a boron trichloride-containing bomb was connected; and the remaining side tube was provided with an Allihn condenser. To the Allihn condenser was fitted a Dewar type cold finger, and a calcium chloride tube was fitted to the outlet of the cold finger. Through the resulting apparatus was passed dry nitrogen at a rate of 200 ml/min for 4 hours to dry the apparatus inside. In the apparatus were placed 41.2 g of benzonitrile and 300 ml of chlorobenzene which had been dried overnight with anhydrous sodium sulfate. The two cold fingers were filled with dry ice-acetone. Into the apparatus contents being stirred with the stirrer was dropwise added, in 2 hours, 60 g of condensed boron trichloride from a cold finger fitted directly to the three-necked flask. Thereby, a white boron trichloride-benzonitrile adduct was formed. After the completion of the dropwise addition of boron trichloride, the cold finger directly fitted to the three-

necked flask was detached, and 21.5 g of ammonium chloride dried at 110° C. overnight was added. When the resulting suspension was heated at 125° C. for 8 hours, the generation of hydrogen chloride stopped substantially and a brown precipitate was formed. The precipitate was collected by filtration, washed with 100 ml of chlorobenzene, and dried under vacuum to obtain 27 g (yield: 79%) of a boron nitride precursor.

10 g of the boron nitride precursor was dissolved in 200 ml of DMF. 100 ml of the DMF was removed from the resulting solution by vaporization, to obtain a uniform viscous solution. The solution was discharged into dry air at 25° C. from a spinning nozzle having holes of 60 µm in diameter, by applying a back pressure of 15 kg/cm<sup>2</sup>, followed by winding-up, to obtain a continuous boron nitride precursor fiber having a diameter of about 20 µm. At this time, the spinning solution had a viscosity of  $2.9 \times 10^4$  poises and the spinning speed was 1.8 m/min.

The boron nitride precursor fiber obtained above was heat-treated in the same manner as in Example 1, at 400° C. in a nitrogen current and then at 1,000° C. in an ammonia gas atmosphere, whereby a non-oriented boron nitride fiber having a diameter of about 15 µm was obtained.

The non-oriented boron nitride fiber was subjected to an orientation treatment in the same manner as in Example 3. The elongation ratio after the orientation treatment was 20.2%. The boron nitride fiber obtained had a degree of orientation of 0.82 and a tensile strength of 1,910 MPa.

#### Example 13

In a three-necked flask having a capacity of 1 l. the center tube was provided with a stirrer; one of the side tubes was provided with a Dewar type cold finger to which a boron trichloride-containing bomb was connected; and the remaining side tube was provided with an Allihn condenser. To the Allihn condenser was fitted a Dewar type cold finger, and a calcium chloride tube was fitted to the outlet of the cold finger. Through the resulting apparatus was passed dry nitrogen at a rate of 200 ml/min for 4 hours to dry the apparatus inside. In the apparatus were placed 41.2 g of acrylonitrile and 300 ml of chlorobenzene which had been dried overnight with anhydrous sodium sulfate. The two cold fingers were filled with dry ice-acetone. Into the apparatus contents being stirred with the stirrer was dropwise added, in 2 hours, 60 g of condensed boron trichloride from a cold finger fitted directly to the three-necked flask. Thereby, a white boron trichloride-acrylonitrile adduct was formed. After the completion of the dropwise addition of boron trichloride, the cold finger directly fitted to the three-necked flask was detached, and 21.5 g of ammonium chloride dried at 110° C. overnight was added. When the resulting suspension was heated at 125° C. for 8 hours, the generation of hydrogen chloride stopped substantially and a brown precipitate was formed. The precipitate was collected by filtration, washed with 100 ml of chlorobenzene, and dried under vacuum to obtain 24 g (yield: 77%) of a boron nitride precursor.

10 g of the boron nitride precursor was dissolved in 200 ml of DMF. 100 ml of the DMF was removed from the resulting solution by vaporization, to obtain a uniform viscous solution. The solution was discharged into dry air at 25° C. from a spinning nozzle having holes of 60 µm in diameter, by applying a back pressure of 15 kg/cm<sup>2</sup>, followed by winding-up, to obtain a continuous boron nitride precursor fiber having a diameter of about 20 µm. At this time, the spinning solution had a viscosity of  $2.9 \times 10^4$  poises and the spinning speed was 1.8 m/min.

The boron nitride precursor fiber obtained above was heat-treated in the same manner as in Example 1, at 400° C. in a nitrogen current and then at 1,000° C. in an ammonia gas atmosphere, whereby a non-oriented boron nitride fiber having a diameter of about 15 µm was obtained.

The non-oriented boron nitride fiber was subjected to an orientation treatment in the same manner as in Example 3. The elongation ratio after the orientation treatment was 20.1%. The boron nitride fiber obtained had a degree of orientation of 0.81 and a tensile strength of 1,890 MPa.

#### Example 14

10 g of the boron nitride precursor produced in the same manner as in Example 1 and 0.05 g of a polyacrylonitrile having a weight-average molecular weight of 500,000 were dissolved in 200 ml of DMF. 100 ml of the DMF was removed from the resulting solution by vaporization, to obtain a uniform viscous solution. The solution was discharged into dry air at 25° C. from a spinning nozzle having holes of 60 µm in diameter, by applying a back pressure of 15 kg/cm<sup>2</sup>, followed by winding-up, to obtain a continuous boron nitride precursor fiber having a diameter of about 20 µm. At this time, the spinning solution had a viscosity of  $6 \times 10^4$  poises and the spinning speed was 18.0 m/min.

25 The boron nitride precursor fiber was subjected to temperature elevation from room temperature to 400° C. at a rate of 1° C./min in a nitrogen current, and then allowed to cool to room temperature, whereby a heat treatment was conducted. The resulting fiber was then subjected to temperature elevation from room temperature to 1,000° C. at a rate of 2° C./min in an ammonia gas atmosphere, then cooled to 500° C. at a rate of 5° C./min, and allowed to cool to room temperature, whereby a heat treatment was conducted. As a result, a non-oriented boron nitride fiber having a diameter of about 15 µm was obtained.

35 The non-oriented boron nitride fiber was subjected to an orientation treatment in the same manner as in Example 3. The elongation ratio after the orientation treatment was 20.2%. The boron nitride fiber obtained had a degree of orientation of 0.82 and a tensile strength of 1,900 MPa.

We claim:

1. A boron nitride fiber comprising boron nitride having a multi-layered structure consisting of planes (C planes) each formed by linkage of 6-membered rings in the plane, in which boron and nitrogen are positioned alternately and bonded to each other, which fiber has a tensile strength of at least 1,400 MPa.
2. A boron nitride fiber according to claim 1, having a tensile strength of at least 1,660 MPa.
3. A boron nitride fiber according to claim 1, having a tensile strength of at least 1,870 MPa.
4. A boron nitride fiber according to claim 1, having a tensile strength of at least 1,890 MPa.
5. A boron nitride fiber according to claim 1, having a tensile strength of at least 1,910 MPa.
6. A boron nitride fiber according to claim 1, having a tensile strength of at least 1,970 MPa.
7. A boron nitride fiber according to claim 1, having a tensile strength of at least 2,300 MPa.
8. A boron nitride fiber comprising boron nitride having a multi-layered structure consisting of planes (C planes) each formed by linkage of 6-membered rings in the plane, in which boron and nitrogen are positioned alternately and bonded to each other, which fiber has a degree of orientation of at least 0.74.
9. A boron nitride fiber according to claim 8, wherein the fiber has a degree of orientation of at least 0.78.

10. A boron nitride fiber according to claim 8, wherein the fiber has a degree of orientation of at least 0.80.

11. A boron nitride fiber according to claim 8, wherein the fiber has a degree of orientation of at least 0.81.

12. A boron nitride fiber according to claim 8, wherein the fiber has a degree of orientation of at least 0.82.

13. A boron nitride fiber according to claim 8, wherein the fiber has a degree of orientation of at least 0.83.

14. A boron nitride fiber according to claim 8, wherein the fiber has a degree of orientation of at least 0.86.

15. A process for producing a boron nitride fiber comprising boron nitride having a multi-layered structure consisting of planes (C planes) each formed by linkage of 6-membered rings in the plane, in which boron and nitrogen are positioned alternately and bonded to each other, which fiber has a tensile strength of at least 1,400 MPa, which process comprises:

- (a) reacting a boron trihalide-nitrile compound adduct with an ammonium halide or a primary amine hydrohalide in the presence of a boron trihalide to form a boron nitride precursor,
- (b) dissolving the boron nitride precursor in a solvent to prepare a boron nitride precursor solution,
- (c) spinning the boron nitride precursor solution to form a boron nitride precursor fiber,
- (d) preheating the boron nitride precursor fiber in an inert gas atmosphere at 100°-600° C.,
- (e) treating the preheated fiber by ammonia in an ammonia gas atmosphere at 200°-1,300° C., and
- (f) heating the fiber treated by ammonia in an inert gas atmosphere at 1,600°-2,300° C. with a tensile stress being applied to the fiber.

16. A process for producing a boron nitride fiber according to claim 15, wherein in the step (a), the boron trihalide is boron trichloride, the nitrile compound is acetonitrile, and the ammonium halide or the primary amine hydrohalide is ammonium chloride.

17. A process for producing a boron nitride fiber according to claim 15, wherein in the step (f), the ammonia-treated fiber is stretched at an elongation ratio of at least 12.7%.

18. A process for producing a boron nitride fiber according to claim 15, wherein in the step (f), the ammonia-treated fiber is stretched at an elongation ratio of at least 15.7%.

19. A process for producing a boron nitride fiber according to claim 15, wherein in the step (f), the ammonia-treated fiber is stretched at an elongation ratio of at least 20.1%.

20. A process for producing a boron nitride fiber according to claim 15, wherein in the step (f), the ammonia-treated fiber is stretched at an elongation ratio of at least 24.7%.

21. A process for producing a boron nitride fiber comprising boron nitride having a multi-layered structure consisting of planes (C planes) each formed by linkage of 6-membered rings in the plane, in which boron and nitrogen are positioned alternately and bonded to each other, which fiber has a tensile strength of at least 1,400 MPa, which process comprises:

- (a) reacting a boron trihalide-nitrile compound adduct with an ammonium halide or a primary amine hydrohalide in the presence of a boron trihalide to form a boron nitride precursor,
- (b) dissolving the boron nitride precursor and an acrylonitrile polymer in a solvent to prepare a boron nitride precursor solution,
- (c) spinning the boron nitride precursor solution to form a boron nitride precursor fiber,
- (d) preheating the boron nitride precursor fiber in an inert gas atmosphere at 100°-600° C.,

(e) treating the preheated fiber by ammonia in an ammonia gas atmosphere at 200°-1,300° C., and

(f) heating the fiber treated by ammonia in an inert gas atmosphere at 1,600°-2,300° C. with a tensile stress being applied to the fiber.

22. A process for producing a boron nitride fiber according to claim 21, wherein in the step (a), the boron trihalide is boron trichloride, the nitrile compound is acetonitrile, and the ammonium halide or the primary amine hydrohalide is ammonium chloride.

23. A process for producing a boron nitride fiber according to claim 21, wherein in the step (b), the acrylonitrile polymer is a polyacrylonitrile.

24. A process for producing a boron nitride fiber according to claim 21, wherein in the step (f), the ammonia-treated fiber is stretched at an elongation ratio of at least 12.7%.

25. A process for producing a boron nitride fiber according to claim 21, wherein in the step (f), the ammonia-treated fiber is stretched at an elongation ratio of at least 15.7%.

26. A process for producing a boron nitride fiber according to claim 21, wherein in the step (f), the ammonia-treated fiber is stretched at an elongation ratio of at least 20.1%.

27. A process for producing a boron nitride fiber according to claim 21, wherein in the step (f), the ammonia-treated fiber is stretched at an elongation ratio of at least 24.7%.

28. A process for producing a boron nitride fiber comprising boron nitride having a multi-layered structure consisting of planes (C planes) each formed by linkage of 6-membered rings in the plane, in which boron and nitrogen are positioned alternately and bonded to each other, which fiber has a degree of orientation of at least 0.74, which process comprises:

- (a) reacting a boron trihalide-nitrile compound adduct with an ammonium halide or a primary amine hydrohalide in the presence of a boron trihalide to form a boron nitride precursor,
- (b) dissolving the boron nitride precursor in a solvent to prepare a boron nitride precursor solution,
- (c) spinning the boron nitride precursor solution to form a boron nitride precursor fiber,
- (d) preheating the boron nitride precursor fiber in an inert gas atmosphere at 100°-600° C.,
- (e) treating the preheated fiber by ammonia in an ammonia gas atmosphere at 200°-1,300° C., and
- (f) heating the fiber treated by ammonia in an inert gas atmosphere at 1,600°-2,300° C. with a tensile stress being applied to the fiber.

29. A process for producing a boron nitride fiber according to claim 28, wherein in the step (a), the boron trihalide is boron trichloride, the nitrile compound is acetonitrile, and the ammonium halide or the primary amine hydrohalide is ammonium chloride.

30. A process for producing a boron nitride fiber according to claim 28, wherein in the step (f), the ammonia-treated fiber is stretched at an elongation ratio of at least 12.7%.

31. A process for producing a boron nitride fiber according to claim 28, wherein in the step (f), the ammonia-treated fiber is stretched at an elongation ratio of at least 15.7%.

32. A process for producing a boron nitride fiber according to claim 28, wherein in the step (f), the ammonia-treated fiber is stretched at an elongation ratio of at least 20.1%.

33. A process for producing a boron nitride fiber according to claim 28, wherein in the step (f), the ammonia-treated fiber is stretched at an elongation ratio of at least 24.7%.

34. A process for producing a boron nitride fiber comprising boron nitride having a multi-layered structure con-

## 31

sisting of planes (C planes) each formed by linkage of 6-membered rings in the plane, in which boron and nitrogen are positioned alternately and bonded to each other, which fiber has a degree of orientation of at least 0.74, which process comprises:

- (a) reacting a boron trihalide-nitrile compound adduct with an ammonium halide or a primary amine hydrohalide in the presence of a boron trihalide to form a boron nitride precursor.
- (b) dissolving the boron nitride precursor and an acrylonitrile polymer in a solvent to prepare a boron nitride precursor solution.
- (c) spinning the boron nitride precursor solution to form a boron nitride precursor fiber.
- (d) preheating the boron nitride precursor fiber in an inert gas atmosphere at 100°–600° C..
- (e) treating the preheated fiber by ammonia in an ammonia gas atmosphere at 200°–1,300° C., and
- (f) heating the fiber treated by ammonia in an inert gas atmosphere at 1,600°–2,300° C. with a tensile stress being applied to the fiber.

## 32

35. A process for producing a boron nitride fiber according to claim 34, wherein in the step (a), the boron trihalide is boron trichloride, the nitrile compound is acetonitrile, and the ammonium halide or the primary amine hydrohalide is ammonium chloride.

36. A process for producing a boron nitride fiber according to claim 34, wherein in the step (b), the acrylonitrile polymer is a polyacrylonitrile.

37. A process for producing a boron nitride fiber according to claim 34, wherein in the step (f), the ammonia-treated fiber is stretched at an elongation ratio of at least 12.7%.

38. A process for producing a boron nitride fiber according to claim 34, wherein in the step (f), the ammonia-treated fiber is stretched at an elongation ratio of at least 15.7%.

39. A process for producing a boron nitride fiber according to claim 34, wherein in the step (f), the ammonia-treated fiber is stretched at an elongation ratio of at least 20.1%.

40. A process for producing a boron nitride fiber according to claim 34, wherein in the step (f), the ammonia-treated fiber is stretched at an elongation ratio of at least 24.7%.

\* \* \* \* \*